

May 22, 1973

D. S. KOZAK ET AL

3,734,714

PROCESS FOR PRODUCING A Co-Ba Al-Si-CONTAINING ALLOY

Filed Sept. 29, 1970



INVENTORS

Donald S. Kozak  
David P. Miller  
BY *Constance T. Bane*  
ATTORNEY

1

3,734,714

## PROCESS FOR PRODUCING A Ca-Ba-Al-Si-CONTAINING ALLOY

Donald S. Kozak, North Tonawanda, N.Y., and David P. Miller, Marietta, Ohio, assignors to Union Carbide Corporation, New York, N.Y.

Filed Sept. 29, 1970, Ser. No. 76,466  
Int. Cl. C22d 7/06

U.S. CL. 75—10 R

9 Claims

### ABSTRACT OF THE DISCLOSURE

This invention relates to a continuous process and apparatus for producing a steel treating agent of a Ca-Ba-Al-Si-containing alloy and particularly to an intermediate pre-chilling step whereby the slag from a molten Ca-Ba-Si-containing alloy is effectively removed prior to introducing the additives of aluminum and a metal selected from the group consisting of iron, nickel, chromium, cobalt and manganese, to form the Ca-Ba-Al-Si-containing alloy.

### BACKGROUND OF THE INVENTION

#### Field of the invention

This invention relates to a continuous process and apparatus for producing a Ca-Ba-Al-Si-containing alloy which can be used as a deoxidizing and cleansing agent to retard the formation of residual inclusions in high quality steels. More particularly, the present invention is directed to an intermediate prechilling step for effectively and economically removing the slag from a conventionally prepared molten Ca-Ba-Si-containing alloy prior to introducing the additives of aluminum and a metal, such as iron, to form a Ca-Ba-Al-Si-containing alloy.

#### Description of the prior art

A calcium-barium-aluminum-silicon-containing alloy is presently being used as an addition agent for treating steels. This aluminum-containing agent retards the formation of residual inclusions in high quality steels thus making the steels usable for precision fabricated parts such as ball bearings and the like. The usual technique for producing this addition agent is to initially prepare, in a submerged arc furnace, an alloy consisting essentially of about 13 to 20% calcium, about 55 to 65% silicon, about 13 to 20% barium and up to 10% iron and/or aluminum.

In preparing this Ca-Ba-Si-containing alloy from commercially available charges of these elements, a slag composed essentially of calcium-barium-silicate



and having approximately the same density as the alloy at the tapping temperature of the arc furnace, which is about 250 lbs./ft.<sup>3</sup> at about 1800° C., is intermixed with the alloy. This contaminated alloy is in a state not amenable for the acceptance of additional charges of aluminum and a metal to produce an overall chemistry which renders the alloy suitable for use as an agent for treating steels. The closeness of the densities between this Ca-Ba-Si-containing alloy and the slag makes impractical the conventional skimming and back-pouring techniques usually employed for separating slag from molten metals. Consequently it is necessary to cool or freeze the slag and Ca-Ba-Si-containing alloy mixture in chills or the like, whereupon during the initial cooling period the slag becomes more viscous than the alloy and settles to the bottom of the chills. Thereafter the slag layer is mechanically or manually removed by conventional means and the Ca-Ba-Si-containing alloy layer is then crushed into small sizes. The sized alloy is next fed into a furnace, such as an induction furnace, where it is heated to a temperature of about 1150° C. Additives of aluminum and a metal such as iron are then

2

introduced in precalculated amounts, with or without additional fines of a Ba-Ca-Si-containing alloy, so as to regulate the chemistry of the overall composite to produce an alloy consisting essentially of about 17-24% aluminum, about 37-43% silicon, about 8-13% barium, about 9-14% calcium, and up to about 25% of at least one metal selected from a group consisting of iron, manganese, nickel, chromium and cobalt; preferably iron.

The Ca-Ba-Al-Si-containing alloys is then tapped into chills or the like where it solidifies, after which it is crushed by conventional techniques into usable sizes.

The separate handling of the Ca-Ba-Si-containing alloy along with the expense of operating a furnace to remelt it increases the overall cost of producing this steel treating agent.

It is the object of this invention to provide a process for separating the slag from the Ca-Ba-Si-containing alloy while the mixture is still in the molten state so that the aluminum and metal additives can be incorporated directly into the molten Ca-Ba-Si-containing alloy thereby avoiding the necessity and expense of a separate remelt step as described above.

### SUMMARY OF THE INVENTION

This invention relates to a continuous process and apparatus for economically producing a steel treating agent of a Ca-Ba-Al-Si-containing alloy consisting essentially of about 8-13% barium, about 9-14% calcium, about 17-24% aluminum, about 37-43% silicon and up to about 25% of at least one metal selected from a group consisting of iron, nickel, chromium, cobalt and manganese. A Ca-Ba-Si alloy containing about 13-20% calcium, about 13-20% barium, about 55-65% silicon and up to 10% iron and/or aluminum is initially produced in a submerged arc furnace by conventional techniques using commercially available charges of these elements. The Ca-Ba-Si-containing alloy intermixed with slag is tapped from the furnace at a temperature of between about 1500° C. and about 2100° C., preferably about 1800° C. Since approximate equality of the densities of the slag and the alloy prevents conventional separation therebetween at this temperature, the molten composite is tapped onto a downwardly inclined prechill runner composed of a refractory material such as sand, brick, graphite or the like. The runner consists of an initially straight segment followed by a second segment containing at least one barrier or projection in the path of the flow to trap, by dam-like means, a portion of the molten composite. The initially straight segment of the runner is designed to permit the cooling of the tapped molten alloy and slag composite to between about 1150° C. and about 1700° C. from the tap temperature which is about 1800° C. Within this temperature range, the slag component of the gravity flowing composite becomes more viscous than the alloy and begins to settle to the bottom of the flow while the alloy rises to the surface. Upon reaching the first barrier, the gravity flow of the composite encounters its first obstacle in which a portion of the lower or bottom layer of the composite containing the slag is trapped while the upper or top layer of the composite, containing substantially the alloy, continues to flow over the barrier. The height of the barrier is calculated so as to trap the slag while providing little or no impedance to the flow of the top layer of the composite containing the Ca-Ba-Si-containing alloy.

To increase the degree of separation between the slag and alloy components, additional barriers may be provided in the path of the flow until a predetermined grade of purity of the Ca-Ba-Si-containing alloy is obtained. The temperature, however, can not be permitted to get lower than about 1100° C. since at this value the alloy becomes viscous and will not flow easily.

The degree of incline of the prechill runner is variable and depends on the length of the initially straight segment of the runner and the height of the barrier or barriers on the second segment. For example, a short initially straight segment for the runner will require a slope which is less than that required for a longer length straight segment since the tapped molten composite will have to be cooled to a degree necessary to have the slag become more viscous than the alloy. Likewise, the height of the barriers also influences the degree of slope of the runner since if the barrier is too low and the slope is high, the slag will not be trapped. The criticality of the runner with respect to length, slope and the height of the barriers thereon is that they be adjusted so that during the initial flow of the tapped molten composite, the cooling of the composite will be sufficient to allow the slag component to become more viscous thereby enabling the first and possible subsequent barrier to effectively trap the slag.

The relatively pure Ca-Ba-Si-containing alloy at the end of the runner is fed into a preheated insulated ladle at a temperature between about 1150° C. and about 1700° C., preferably about 1300° C., where it is then weighed. The required amount of aluminum and a metal, such as iron, necessary to adjust the chemistry of the alloy to the range given above is calculated and then added to the ladle. In some cases fines of a Ca-Ba-Si-containing alloy and/or a Ba-Ca-Al-Si-containing alloy, or calcium metal or a calcium-containing alloy may be required to further adjust the chemistry of the overall composite to produce a Ba-Ca-Al-Si-containing alloy consisting essentially of about 8-13% barium, about 9-14% calcium, about 17-24% aluminum, about 37-43% silicon and up to 25% of a metal such as iron. An inert gas, such as argon or nitrogen, introduced by a graphite tube from the top, or from a porous plug at the bottom, can be used to stir the alloy for about 3 minutes after all additions are made, such time period being sufficient to substantially homogenize the alloy. Thereafter the alloy, at a temperature between about 1100° C. and about 1250° C., is cast into chills and allowed to cool to ambient. The alloy is then crushed by conventional techniques and appropriately sized for use.

Not only is the remelting step of the Ca-Ba-Si-containing alloy dispensed with, but the formerly wasted superheat of this alloy in its initial production is now utilized to aid in the melting and alloying of the aluminum and metal additives in the Ba-Ca-Al-Si-containing alloy.

It is also to be understood that aluminum and/or a metal, such as iron, could be preheated in the ladle before the Ca-Ba-Si-containing alloy is fed into the ladle, or that aluminum and/or iron could be introduced into the ladle in the molten state after the introduction of the Ca-Ba-Si-containing alloy. Since the reaction of iron with silicon in a silicon-containing alloy is an exothermic reaction and the alloying of aluminum into the Ca-Ba-Si-containing alloy is an endothermic reaction, then the adding of each can be varied to maintain the temperature within the ladle at some desired range.

The single drawing shows a sectional view of a side elevation of a prechill runner for use in implementation of this invention.

In the drawing a submerged arc furnace 1, electrode not shown, has a tap hole 11 through which a molten composite 12 of slag 8 and Ca-Ba-Si-containing alloy 9 is tapped. Slag 8 is indicated by short line segments and Ca-Ba-Si-containing alloy 9 is shown as small circles. The somewhat intermixed molten composite 12 is tapped onto a downwardly inclined runner 13 having a straight segment 2 forming an angle B between about 20° and about 60°, preferably about 45°, with reference to the horizontal. Segment 3 of runner 13 has a slope A between about 10° and about 30°, preferably about 15°, with reference to the horizontal and has barriers 4, 5, and 6

projecting upward from its top surface 10. During the initial gravity flow of molten composite 12 upon segment 2 of runner 13, the composite 12 cools to a degree whereupon slag 8 becomes more viscous than alloy 9 and begins to settle to the bottom of composite 12. Upon reaching barrier 4, the portion of slag 8 at the bottom of composite 12 is trapped in cavity 14. The flow of composite 12 is next interrupted by barriers 5 and 6, whereupon an additional amount of slag 8 is trapped in cavities 15 and 16, respectively. The relatively slag-free composite 12 accumulates in cavity 17, whereupon the substantially pure Ca-Ba-Si-containing alloy, at a temperature between about 1100° C. and about 1700° C., spills over projection 7 into a preheated ladle 18. At this stage of the process, aluminum, a metal such as iron, and/or fines of Ca-Ba-Si-containing alloy or Ca-Ba-Si-Al-containing alloy are added thereto or some elements thereof are in the ladle 18 prior to the introduction of the molten Ca-Ba-Si-containing alloy. An inert gas is introduced through porous plug 19 to stir and homogenize the alloy therein. The Ca-Ba-Al-Si-containing alloy is then cast into chills for cooling to ambient and thereafter the solidified alloy is crushed into usable sizes. Any Ca-Ba-Si-containing alloy remaining on the runner can be separated from the slag by conventional techniques and remelted or used as an additive to adjust the chemistry of the alloy in the ladle.

It should be realized that the runner shown in the drawing is for illustrative purposes and various designs and contour are feasible. For example, segment 2 and segment 3 can be disposed with the same slope without departing from the invention.

#### EXAMPLE

A 13,000 kilowatt submerged arc furnace was used to conventionally produce 5000 lbs. of Ca-Ba-Si-containing alloy which had slag intermixed therewith. A molded sand runner, similar to the one shown in the drawing, was positioned adjacent to the tap hole of the furnace. The horizontal length of the runner was 30 feet with the straight segment being 12 feet, at a slope of 45°, and the barrier-containing segment being 18 feet, with a slope of 15°. The height of the barrier measured from the lowest point in the cavities was 1.5 feet. A 67 cubic foot ladle was positioned at the end of the runner and was equipped with a graphite tube for introducing nitrogen gas.

Alloy and slag from the furnace were tapped onto the runner and gravity-fed into the ladle. The tapping temperature, weight, and additions of two heats are shown in Table 1. The molten alloy of the first heat was fed into the ladle at a temperature of 1590° C. and visually indicated no traces of slag. Thereafter 685 lbs. of steel, 150 lbs. of calcium and 1180 lbs. of molten aluminum were introduced which yielded a final temperature of 1410° C. Nitrogen gas was next introduced through a graphite tube in the ladle to stir and homogenize the alloy therein. The stirring continued for 3 minutes after all additions were completed and thereafter the alloy was cast into chills measuring 5' x 5' x 3" for cooling down to ambient. An analysis of the alloy composite before and after the addition of the aluminum, steel and calcium is shown in Table 2.

The same procedure was undertaken for heat 2 except that 250 lbs. of steel was in the ladle prior to the introduction of the molten alloy from the runner. With the temperature of the steel and Ca-Ba-Si-containing alloy in the ladle at 1455° C., an additional 500 lbs. of steel, 150 lbs. of calcium, 1390 lbs. of aluminum, and 360 lbs. of Ca-Ba-Si-Al-containing fines were added. This gave a final temperature of 1280° C. Nitrogen gas was again introduced to stir the alloy and was continued for 3 minutes after all additions were made. The alloy was thereafter cast into chills as specified above and an analysis of the alloy is likewise shown in Table 2.

TABLE 1

| Heat   | Tapping temp., (° C.) |             | Weight, lbs. |             | Additions, lbs. |       |       | Alloy fines |
|--------|-----------------------|-------------|--------------|-------------|-----------------|-------|-------|-------------|
|        | From furnace          | From runner | From furnace | From runner | Ca              | Steel | Al    |             |
| 1----- | 1,800                 | 1,590       | 5,000        | 3,580       | 150             | 685   | 1,180 | -----       |
| 2----- | 1,800                 | 1,455       | 5,000        | 3,920       | 150             | 750   | 1,390 | 360         |

TABLE 2

| Heat                                               | Ca   | Ba   | Si   | Fe   | Al    | Traces of   |  |
|----------------------------------------------------|------|------|------|------|-------|-------------|--|
|                                                    |      |      |      |      |       | O, N, C, Cr |  |
| Analysis of Ca-Ba-Si-containing alloy (percent)    |      |      |      |      |       |             |  |
| 1-----                                             | 15.9 | 16.6 | 59.8 | 6.3  | ----- | 1.4         |  |
| 2-----                                             | 16.1 | 16.0 | 60.6 | 5.7  | ----- | 1.6         |  |
| Analysis of Ca-Ba-Si-Al-containing alloy (percent) |      |      |      |      |       |             |  |
| 1-----                                             | 11.2 | 10.3 | 39.4 | 16.4 | 20.6  | 2.1         |  |
| 2-----                                             | 11.5 | 10.1 | 39.7 | 16.8 | 20.7  | 1.2         |  |

## What is claimed is:

1. A process for making an aluminum-containing alloy addition agent consisting essentially of about 17-24% aluminum, about 37-43% silicon, about 8-13% barium, about 9-14% calcium and up to 25% of at least one of the metals selected from a group consisting of iron, nickel, manganese, chromium and cobalt, comprising:
  - (a) preparing a molten Ca-Ba-Si-containing alloy in a submerged arc furnace at an elevated temperature wherein slag is intermixed with the alloy;
  - (b) tapping said slag containing Ca-Ba-Si alloy onto a downwardly inclined runner, said runner having an initially straight segment followed by a second segment containing at least one barrier projecting upward from the surface into the flow path on said runner so as to form a cavity on said runner;
  - (c) cooling said slag containing Ca-Ba-Si-alloy to a temperature at which the slag becomes more viscous than the Ca-Ba-Si-containing alloy whereupon said slag settles at the bottom of the flow while the alloy rises to the top;
  - (d) partially obstructing the gravity flow of said slag containing Ca-Ba-Si alloy by said barrier so as to trap said slag in the cavity formed by said barrier while allowing the alloy at the upper portion of the flow to continue;
  - (e) collecting said relatively slag-free Ca-Ba-Si-containing alloy in a ladle;
  - (f) mixing said Ca-Ba-Si-containing alloy with an additive consisting of aluminum and at least one of the metals selected from the group consisting of iron, nickel, chromium, calcium, manganese and cobalt

in said ladle to form an aluminum-containing alloy; and

(g) casting said aluminum-containing alloy.

2. The process of claim 1 wherein at least one of the additives in step (f) is in the ladle prior to introducing the relatively slag-free Ca-Ba-Si-containing alloy.

3. The process of claim 2 wherein at least one of the additives in step (f) is added to the ladle after the introduction of the relatively slag-free Ca-Ba-Si-containing alloy.

4. The process of claim 1 wherein at least one of the additives in step (f) is added to the ladle in the molten state.

5. The process of claim 1 where the mixing in step (f) is accomplished by introducing an inert gas into the ladle.

6. The process as in claim 1 wherein in step (b) the slag-containing Ca-Ba-Si alloy is tapped at a temperature between about 1500° C. and about 2100° C.

7. The process as in claim 6 wherein in step (c) the slag-containing Ca-Ba-Si alloy is cooled to a temperature between about 1150° C. and about 1700° C.

8. The process of claim 7 wherein in step (e) the relatively slag-free Ca-Ba-Si alloy is collected in the ladle at a temperature about 1300° C.

9. The process of claim 1 wherein a calcium-containing alloy is added to the ladle in step (f) to adjust the chemistry of the aluminum-containing alloy.

## References Cited

## UNITED STATES PATENTS

- 40 3,321,300 5/1967 Worner ----- 75-93 R  
 2,519,593 8/1950 Offenhaver ----- 266-34 PT  
 1,862,787 6/1932 Error ----- 266-38

## FOREIGN PATENTS

- 45 643,325 6/1962 Canada ----- 75-93 R  
 933,393 8/1963 Great Britain ----- 75-134

WINSTON A. DOUGLAS, Primary Examiner

M. J. ANDREWS, Assistant Examiner

U.S. CL. X.R.

75-63, 93 R, 134 A, 134 S; 164-134; 266-37, 38